

**1**

2,745,770

**ORGANIC SHAPED STRUCTURES COATED WITH WERNER-TYPE CHROMIUM COMPOUNDS AND METHOD OF MAKING THE SAME**

Richard W. Kingerley, Jr., Wilmington, Del., assignor to  
E. I. du Pont de Nemours and Company, Wilmington,  
Del., a corporation of Delaware

No Drawing. Application April 9, 1952,  
Serial No. 281,481

4 Claims. (Cl. 117—139.5)

This invention relates to shaped structures having improved anti-static properties and to processes for producing the same. More particularly, it relates to films, filaments, fibers, monofil, coatings, fabrics and like structures, having a moisture regain of no greater than five percent and a resistivity of at least  $400,000 \times 10^8$  ohms, the surfaces of which have uniformly distributed thereon as an anti-static agent a complex compound of the Werner type in which trivalent nuclear chromium atoms are coordinated with a monocarboxylic acid selected from the class consisting of p-nitrophenylacetic acid, p-nitrobenzoic acid, phenylacetic acid, trichloroacetic acid, thioglycollic acid, cyanoacetic acid and gluconic acid.

Films, filaments, fibers, monofil, coatings fabrics and like structures having low moisture regain and high resistivity have a propensity to ready develop strong electrostatic charges which make them difficult to manipulate during manufacture, subsequent processing and use, such as, for instance, in the steps of spinning, knitting, weaving, slitting, printing, perforating, winding, sealing, packaging and other finishing operations. By reason of their highly charged surfaces, these articles also accumulate heavy dust deposits which, of course, are very undesirable.

Then, too, in the manufacture of film for photographic uses having low moisture regain and high resistivity, the discharge of positive and negative charges during processing exposes the light-sensitive silver halides leaving characteristic static marks after development.

Various agents, methods and apparatus have heretofore been proposed to eliminate or at least minimize the accumulation of electrostatic charges on shaped structures without detracting from their physical properties, but they are not entirely satisfactory.

Now I have found that the surface characteristics of films, filaments, fibers, monofil, sheets, coating and like structures having a moisture regain of no greater than 5% and a resistivity in ohms of at least  $400,000 \times 10^8$  can be improved by applying to the surfaces of these structures a Werner type chromium complex in which a trivalent chromium atom is coordinated with a monocarboxylic acid group of the class consisting of p-nitrophenylacetato, p-nitrobenzoato, phenylacetato, trichloroacetato, thioglycollato, cyanoacetato and gluconato; from solutions of such complexes, and thereafter drying said structures by any suitable expedient. These complex compounds are outstanding in that they "wet" the surface of the shaped structure, resulting in a substantially uniform, adherent coating application.

Chromium coordination complex compounds of the Werner type suitable for use in accordance with my invention can be coordinated with any of the aforementioned monocarboxylic acids. A compound of the acid such as an ester or salt which can liberate the free acid under the condition of the coordination reaction is, of course, equivalent to the free acid.

General methods for preparing suitable Werner type chromium acid complexes are described in Iler Patents Nos. 2,273,040, 2,356,161 and 2,524,803. The processes

**2**

described in 2,273,040 and 2,356,161 effect the reaction between a carboxylic acid group and a basic trivalent chromium salt of a monobasic acid in the substantial absence of free water. U. S. 2,524,803 teaches a method whereby contact between the basic chromium chloride and the carboxylic acid group is effected in the presence of alcohol.

The nature of the Werner-type complex chromium compounds and the nomenclature applied to them is described fully in U. S. Patents 2,273,040, 2,356,161 and 2,524,803. By deleting the suffix "-ic" from the name of the carboxylic acid and adding the suffix "-ato" a system of naming the acid groups coordinated with the chromium, and hence for naming the chromium complexes, is provided. Thus, p-nitrophenylacetic acid gives p-nitrophenylacetato groups and the complex is called p-nitrophenylacetato chromic chloride.

The Werner complexes are admixed with a suitable volatile solvent which does not affect the complex, such as, for example, water, methanol, ethanol, isopropanol, t-butanol, aqueous solutions of these alcohols, and butyl acetate.

These solutions should contain from about 0.1% to about 1.0% by weight of the Werner type chromium complex.

Application of the solution of the Werner-type chromium complex to the surface of the structure having a moisture regain of 5% or less and resistivity of at least  $400,000 \times 10^8$  ohms can be accomplished by any convenient expedient which insures intimate contact of the complex with the substrate. For instance, dipping, spraying, brushing, roll coating, paddling, and the like operations may be employed.

The temperature of the "application" bath is not critical but it should be such that the chromium complex is dissolved or thoroughly dispersed. In general, the temperature should be maintained preferably below 100° F.

Aqueous solutions of the Werner type chromium complexes are particularly well suited for purposes of this invention. Should, however, the type of fabric or fiber under treatment be very difficult to wet because of the presence of sizing agents or other contaminates on the surface, it may be necessary to add some isopropanol to the aqueous solution of the complex compound to improve the wetting characteristics, but in most instances this will not be necessary.

The shaped structure treated with an aqueous solution of a chromium complex can be cured on a tenter frame, drum dryers or other suitable apparatus at a temperature of from 140° to 250° F. for a period of about 1 to 5 minutes. Air drying will suffice.

The thickness of the anti-static layer is variable from that just sufficient to form a uniform coherent coating to a maximum thickness determined by the characteristics of the layer. Thus too thick a coating may lead to tackiness or flaking. While the optimum coating weight may vary depending upon coating conditions, a practical range for film is from about 2 to 50 milligrams of complex per square yard of film surface. The preferred coating weight for photographic film is from about 0.15 mg. to 0.35 mg. total solids per square decimeter.

The shaped structures whose surfaces have uniformly distributed thereon a Werner-type chromium complex may be in the form of films, filaments, fibers, monofil, coatings, fabric and the like but they are all characterized by having a moisture regain no greater than 5 per cent and a resistivity of at least  $400,000 \times 10^8$  ohms.

By the term "moisture regain" is meant the per cent moisture in the shaped structure based on a bone-dry basis. This definition is in accord with that used in the art and is fully described by Bruce E. Hartschuk in his

book "Introduction to Textile Chemistry," John Wiley & Sons, Inc., New York, 1950, at pages 118-122.

The American Society for Testing Materials has established a set of standard moisture regains, shown in Table 17 of the aforementioned Hartsuch reference. The per cent moisture regain approximates the per cent of water that each structure would absorb if exposed to an average or normal atmosphere, which is assumed to have a relative humidity of 65% at a temperature of 70° F. In other words, a percentage of moisture regain of 5 means that 5 per cent of water on a bone-dry basis is absorbed by the shaped structure when exposed to an atmosphere having a relative humidity of 65% at a temperature of 70° F.

The term "resistivity" is used in its conventional sense to mean the electrical resistivity of the shaped structures. The apparatus used to determine the electrical resistance of the various structures is fully described by Mason Hayek and F. C. Chromey in volume 40 of American Dyestuff Reporter, at pages 225-227.

The principle involved in the Hayek-Chromey instrument is the measurement of the IR drop in a known resistance, where I is the current leaking thru the sample. The voltage across the standard resistance is amplified with an electrometer tube, and the extent of the unbalance of the circuit is measured with a microammeter. From a graph of the logarithm of the meter deflection against the logarithm of the test resistance in standard resistor units, the unknown resistance can be determined.

Included among the shaped structures which have moisture regains of 5% or less and electrical resistivities of at least  $400,000 \times 10^8$  ohms are polyamides, polyesters, such as for instance polyethylene terephthalate, acrylic polymers, such as for instance polyacrylonitrile, vinyl polymers other than polyvinyl alcohol, vinylidene chloride polymers, vinyl-acrylic copolymers, polystyrene, polyethylene and the like.

The electrostatic voltages of the various shaped structures against synthetic rubber are measured by the method first described by D. J. Lehmicke, American Dyestuff Reporter 38, 853 (1949) and more recently by L. B. Chandler, Textile World 101, 116 (1951). In brief, the method comprises charging the shaped structure such as nylon fabric by rubbing it ten times with a neoprene-gloved hand. The charged structure is then dropped into an aluminum beaker insulated from the ground and connected to a voltmeter. The voltage generated is measured by reading the voltmeter.

The nature of this invention and its method of application will be better understood by reference to the following illustrative examples:

#### Example 1

A strip of film base composed of polyethylene terephthalate having a moisture regain of less than 1% at 65% relative humidity was coated on one surface with a solution having 0.157 part by weight of stock p-nitrophenylacetato chromic chloride and 78.9 parts by weight of ethanol. The coating was dried at a temperature of 160° F. for a period of three minutes. The surface resistivity of the treated film is  $1000 \times 10^8$  ohms.

The surface of a control strip (untreated) of the above polyethylene terephthalate film has a surface resistivity of more than  $10,000,000 \times 10^8$  ohms.

#### Example 2

A film strip composed of polyethylene terephthalate as described in Example 1 is coated on one side with an aqueous solution having the following composition by weight:

|                                              | Parts  |
|----------------------------------------------|--------|
| p-Nitrobenzoato chromic chloride             | 0.156  |
| Wetting agent (alkyl aryl polyether alcohol) | 1.00   |
| Water                                        | 100.00 |

The coating is dried at 160° F. for a period of three minutes. The surface resistivity of the treated film is  $5000 \times 10^8$  ohms. The control untreated film has a surface resistivity of  $>10,000,000 \times 10^8$  ohms.

#### Example 3

A 7 x 9 inch piece of nylon taffeta having a moisture regain of about 3.8% (70° F., 65% R. H.) and a resistivity of greater than  $950,000 \times 10^8$  ohms was coated with an isopropanol solution containing 0.9% by weight of stock p-nitrophenylacetato chromic chloride solution. (By the term "stock p-nitrophenylacetato chromic chloride solution" is meant an isopropanol solution of p-nitrophenylacetato chromic chloride containing about 6% chromium.)

The treated fabric was dried and its electrostatic voltage against synthetic rubber was determined by the aforementioned method of Lehmicke and Chandler. A voltmeter reading of 76 volts (78° F., 72% R. H.) was obtained for the treated fabric. The electrostatic voltage of the nylon control (untreated) generated against synthetic rubber was 760 volts.

The treated nylon taffeta retained 6 mg./sq. ft. of the complex chromium compound.

#### Example 4

A 7 x 9 inch piece of polyethylene terephthalate taffeta having a moisture regain of about 0.4% (65% R. H.) and a resistivity of greater than  $1,000,000 \times 10^8$  ohms was coated with an aqueous solution containing 0.6% by weight of stock p-nitrophenylacetato chromic chloride.

The treated fabric was dried and its electrostatic voltage generated against synthetic rubber was then determined. The treated fabric generated 140 volts against neoprene while the polyethylene terephthalate control fabric generated 960 volts.

The polyester taffeta treated with the p-nitrophenylacetato chromic chloride retained about 4 mg./sq. ft. of the chromium complex.

I claim:

1. A method which comprises applying to an organic shaped structure having a moisture regain of no greater than 5% and a surface resistivity of at least  $400,000 \times 10^8$  ohms a solution containing a complex chromium compound of the Werner type selected from the group consisting of p-nitrophenylacetato chromic chloride, p-nitrobenzoato chromic chloride, phenylacetato chromic chloride, trichloroacetato, thioglycollato, cyanoacetato and gluconato chromic chloride, cyanoacetato chromic chloride and gluconato chromic chloride, and subsequently drying said structure.

2. A method which comprises coating an aqueous solution of a complex compound of the Werner type in which a trivalent nuclear chromium atom is coordinated with a monocarboxylic acid group of the class consisting of p-nitrophenylacetato, p-nitrobenzoato, phenylacetato, trichloroacetato, thioglycollato, cyanoacetato and gluconato groups onto a surface of an organic shaped structure having a moisture regain of no greater than 5% and a surface resistivity of at least  $400,000 \times 10^8$  ohms and subsequently drying said coated structure.

3. A method which comprises coating a solution containing a volatile solvent and a complex compound of the Werner type said complex chromium compound being selected from the group consisting of p-nitrophenylacetato chromic chloride, p-nitrobenzoato chromic chloride, phenylacetato chromic chloride, trichloroacetato chromic chloride, thioglycollato chromic chloride, cyanoacetato chromic chloride, and gluconato chromic chloride, in which a trivalent nuclear chromium atom is coordinated with a monocarboxylic acid group of the class consisting of p-nitrophenylacetato, p-nitrobenzoato, phenylacetato, trichloroacetato, thioglycollato, cyanoacetato and gluconato groups onto a surface of an organic shaped structure having a moisture regain of no greater than 5% and a sur-

face resistivity of at least  $400,000 \times 10^8$  ohms and drying the coated layer.

4. Organic shaped structures the surfaces of which have uniformly distributed thereon as an anti-static agent a complex chromium compound of the Werner-type, said complex chromium compound being selected from the group consisting of p-nitrophenylacetato chromic chloride, p-nitrobenzoato chromic chloride, phenylacetato chromic chloride, trichloroacetato chromic chloride, thioglycollato chromic chloride, cyanoacetato chromic chloride, and gluconato chromic chloride, said structures having prior to surface application of said chromium compound a moisture regain no greater than 5% and a surface resistivity of at least  $400,000 \times 10^8$  ohms.

15

## References Cited in the file of this patent

## UNITED STATES PATENTS

|    |           |                |       |               |
|----|-----------|----------------|-------|---------------|
| 5  | 2,273,040 | Iler           | ----- | Feb. 17, 1942 |
|    | 2,356,161 | Iler           | ----- | Aug. 22, 1944 |
|    | 2,532,691 | Berry          | ----- | Dec. 5, 1950  |
|    | 2,628,176 | Simon et al.   | ----- | Feb. 10, 1953 |
|    | 2,647,836 | Patten         | ----- | Aug. 4, 1953  |
| 10 | 2,673,824 | Biefeld et al. | ----- | Mar. 30, 1954 |
|    | 2,673,825 | Biefeld et al. | ----- | Mar. 30, 1954 |

## OTHER REFERENCES

Knowlton: Standard Handbook for Electrical Engineers, 7th edition, 1941, sec. 4-595, page 389.